

## UNITED STATES PATENT OFFICE

LOUIS WEISBERG AND WILLARD F. GREENWALD, OF NEW YORK, N. Y., ASSIGNEES TO  
WEISBERG & GREENWALD, INC., OF NEW YORK, N. Y., A CORPORATION OF NEW  
YORK

## CHROMIUM COATED ARTICLES AND METHOD OF PREPARING SAME

No Drawing.

Application filed August 1, 1930. Serial No. 472,487.

This invention relates to the electrodeposition and particularly to the preparation of surfaces to receive a wear-resisting coating of chromium.

5 Lead and lead alloys such as type metal and similar metals which are relatively soft are easily abraded, and consequently the exposed surfaces, when subjected to wear, are rapidly destroyed. This is particularly true 10 in the case of stereotype plates and slugs, which are made by casting a molten alloy of lead containing small amounts of hardening agents such as antimony.

Attempts have been made heretofore to deposit chromium on and thereby to protect 15 soft metals by providing a wear-resisting surface, but it has not been possible to accomplish the deposition of chromium successfully on such materials because the chromium 20 will not adhere to the base metal. The procedure often employed in chromium plating of first depositing a flash coating of copper or nickel does not avoid the difficulty, because copper and nickel do not form a satisfactory 25 bond with metals such as lead, and consequently do not afford a proper base for the chromium.

It is the object of the present invention to provide a simple and effective procedure 30 whereby chromium can be deposited in a simple and satisfactory manner upon a surface of a soft metal such as lead or an alloy thereof to produce a wear-resisting chromium surface which adheres to the underlying 35 metal and affords a surface capable of resisting wear.

Another object of the invention is the provision of a method for depositing chromium satisfactorily on stereotype printing plates 40 and slugs and other similar objects, whether prepared by the stereotype process or otherwise, and the provision also of a printing surface having a type metal base and an adhering coating of chromium thereon.

45 The object of the invention is accomplished by suitably cleaning the surface of the article to be coated and then dipping it into an aqueous bath containing a mercury salt. For this purpose, solutions of mercuric cyanide and 50 sodium cyanide or mercuric chloride and am-

monium chloride are suitable, but other mercury salts may be similarly used. The dipping of the article having an exposed surface of lead or an alloy thereof in the solution of a suitable mercury salt results in the formation of an amalgam of mercury and lead on the surface of the article to be treated.

The surface carrying the lead-mercury amalgam is then brushed thoroughly until it is clean, and is disposed in a suitable electrolytic bath capable of depositing, through the action of the electric current, a coating of a metal capable of amalgamating with mercury, such as brass, upon the surface. The mercury present in the treated surface amalgamates with the zinc in the brass which is deposited on the surface, thus giving a perfect bond between the base metal and the brass deposit. The surface may be cleaned again and is then ready for the deposition of the chromium, which adheres to and forms a coherent deposit upon the brass coating to afford a hard, wear-resisting surface.

The invention will be described particularly with reference to the treatment of stereotype plates and slugs, although the procedure may be employed for the deposition of chromium upon any article the exposed surface of which consists of a metal capable of amalgamating with mercury. A stereotype plate 80 may be prepared in the usual manner by casting a suitable type metal alloy having a basis of lead in the usual matrix. In the ordinary stereotype process a matrix of paper is employed. The same principle is used, however, in the preparation of linotype and monotype slugs and in the casting of ordinary type.

The stereotype plate, for example, is cleaned carefully to remove any adhering 90 foreign materials and is then dipped into an aqueous bath containing for example 8 to 10 grams per liter of mercuric cyanide with 60 grams per liter of sodium cyanide, or 7.5 grams per liter of mercuric chloride with the 95 addition of 4 grams per liter of ammonium chloride. The salts of mercury mentioned are best adapted for the practice of the invention, but others may be utilized. The dipping of the plate in the mercury bath results imme- 100

diately in the formation of the film of lead amalgam on the surface of the plate. The surface is brushed thoroughly to remove any foreign particles adhering thereto and is then 5 plated with brass.

We may employ any suitable brass plating procedure such as that set forth, for example, in "Principles of Electroplating and Electro-forming" by Blum and Hogaboam, 2nd edition, pages 379-389. Thus, we may employ 10 a cyanide solution containing copper and zinc in the ratio of 80:20, with a total metal content of at least 22.5 grams per liter and a free cyanide content about one-fourth the total 15 of combined cyanide. To this bath may be added from 30 to 60 grams per liter of sodium carbonate. In this electrolyte, at a temperature of about 40° C., the surface to be coated may be disposed as the cathode and subjected 20 to the electric current with a cathode current density of about 2.8 amperes per sq. ft. We thus provide on the surface of the article to be coated a coating of brass in which the zinc is amalgamated with the lead amalgam 25 previously formed on the surface, affording a perfect bond with the underlying metal. After a suitable interval which is best determined by consideration of the amount of brass to be deposited on the surface, the cathode is removed and is again thoroughly 30 cleaned. It is ready then for the deposit of chromium.

For the chromium plating, we prefer to employ the well-known Sargent solution containing, for example, from about 250 to 450 35 grams per liter of chromic acid ( $\text{CrO}_3$ ) and from 2.5 to 4.5 grams per liter of sulphate radical represented by the addition to the chromic acid of sulphuric acid, chromium 40 sulphate or an alkali sulphate such as sodium sulphate. The plate having the brass coating is disposed as the cathode in this solution, which is maintained at a temperature preferably between 30 and 45° C. It is subjected to 45 the electric current at a cathode current density of, for example, 1 ampere per sq. in., for a brief period, sufficient to deposit a layer of chromium of the required thickness upon the surface of the plate. The chromium is 50 deposited as a bright, dense and coherent layer and affords a hard, wear-resisting surface. It bonds perfectly with the underlying coating of brass and consequently will not flake when pressure is applied in the printing 55 operation, nor is it affected by the abrasive or corrosive properties of the ink employed in printing.

In fact, it has been found that printing plates of lead or alloys thereof, when prepared and coated with chromium in the manner described, will remain sharp and clear and show no evidence of wear after producing many times the number of impressions which can be obtained ordinarily from the 65 type metal surface.

While the invention has been described with reference more particularly to the deposition of chromium on lead and alloys thereof, it may be employed also to similarly coat other metals and alloys thereof which are capable of forming amalgams, for example, zinc and zinc alloys such as die casting alloys. 70

It is to be understood that the details of plating with brass and with chromium form no part of the present invention and are subject to variation, the procedures described being merely typical of those well known in the art and adapted for the purpose of the invention. The word "brass" as used in the following claims is to be understood as including equivalent alloys and metals capable of forming amalgams. The words "lead-containing metal" are to be understood to include equivalent alloys and 85 metals capable of forming amalgams. 90

Various changes may be made in the details of the procedure without departing from the invention or sacrificing the advantages thereof. 95

We claim:

1. The method of preparing a surface of lead-containing metal for chromium plating which comprises forming on the surface a layer of lead amalgam and electrolytically 95 depositing brass thereon.

2. The method of coating with chromium a surface containing a metal capable of forming an amalgam which comprises subjecting the surface to a solution of a mercury compound, depositing a layer of brass on the surface and then depositing a layer of chromium thereon. 100

3. A printing element having an underlying support of lead-containing metal, a surface of chromium and an intermediate layer of brass bonded to the lead-containing metal by an amalgam. 105

In testimony whereof we affix our signatures. 110

LOUIS WEISBERG.  
WILLARD F. GREENWALD.

115

120

125

130